

## UNITED STATES PATENT OFFICE

WILLIAM E. McCULLOUGH, OF DETROIT, MICHIGAN, ASSIGNOR TO BOHN ALUMINUM & BRASS CORPORATION, OF DETROIT, MICHIGAN, A CORPORATION OF MICHIGAN

## NONCORRODIBLE ALUMINUM ALLOY

No Drawing.

Application filed November 2, 1931. Serial No. 572,740.

The invention relates to aluminum alloys and has for its object the obtaining of a material having the following characteristics:

First, high resistance to corrosion;

5 Second, adaptability to formation by extrusion;

Third, capability of receiving high polish with the production of a non-tarnishing surface of bright luster.

10 In the forming of aluminum alloys copper is quite generally used as a hardening agent but as usually manufactured its presence in the alloy is detrimental to corrosion resistance. I have discovered that by using a

15 boronized copper this tendency to corrosion is very largely overcome. I have also discovered that a small percentage of silicon in the alloy improves its physical characteristics and in the presence of boronized copper is not

20 detrimental to either the color, polishing or anti-corrosive properties of the alloy. Additional elements used in the alloy are chromium and cobalt.

One specific example of my improved alloy 25 is of the following composition:

|                  | Percent |
|------------------|---------|
| Aluminum         | 97.75   |
| Boronized copper | .50     |
| Chromium         | .75     |
| 20 Cobalt        | .25     |
| Silicon          | .75     |

The above formula may be varied and the range of variation permissible includes copper, .5 to 3%; chromium .75 to 1.5%; cobalt .25 to .50% and silicon .75 to 3%.

The material can be readily worked and is especially suited to formation by extrusion. In the extruded condition the specific alloy 40 above described has a tensile strength of 20,000 pounds per square inch or better, an elongation of 35% in two inches and a Brinell hardness of 36 or over.

My improved alloy is particularly adapted 45 for exterior finish of buildings as it is capable of receiving a highly polished surface and will retain its bright luster when exposed to weather. The alloy is also only slightly affected by the standard salt spray test for 50 corrosion resistance.

What I claim as my invention is:

1. An aluminum alloy comprising copper .5 to .8%, chromium .75% to 1.5%, cobalt .25% to .50%, silicon .75% to 3%, and the balance of commercial aluminum.

5 2. An aluminum alloy substantially of the following composition:

|                  | Per cent |
|------------------|----------|
| Boronized copper | .5       |
| Chromium         | .75      |
| Cobalt           | .25      |
| Silicon          | .75      |

and the balance of commercial aluminum.

3. An aluminum alloy containing chromium .75% to 1.5%; cobalt .25% to .50%; silicon .75% to 3%; copper free from any oxide thereof .5% to 3% and the balance of commercial aluminum.

In testimony whereof I affix my signature.

WILLIAM E. McCULLOUGH.

75

80

85

90

95

100